# EUROPEAN PATENT SPECIFICATION

(11) **EP 0 137 180 B1**
(45) Date of publication and mention of the grant of the patent: **28.12.1988**
(21) Application number: 84109194.5
(22) Date of filing: 02.08.1984
(51) Int. Cl.: C22C 1/04, C22C 21/00

(54) **Heat-resisting aluminium alloy**
Hitzebeständige Aluminiumlegierung
Alliage d'aluminium, résistant aux températures élevées

(30) Priority: 17.08.1983 JP 149161/83
(43) Date of publication of application: 17.04.1985
(73) Proprietor: NISSAN MOTOR CO., LTD., Yokohama-shi Kanagawa-ken (JP)
(72) Inventor: Shioda, Masahiko, Hodogaya-ku Yokohama City (JP); Suzuki, Syunsuke, Minato-ku Tokyo (JP); Matsuyama, Akira, Zuchi City (JP); Maki, Yoshishiro, Minamishimoura-cho Miura City (JP)
(74) Representative: Grünecker, Kinkeldey, Stockmair & Schwanhäusser Anwaltssozietät

(56) References cited:
- FR-A- 1 370 542
- GB-A- 498 227
- US-A- 2 966 731
- US-A- 3 265 493
- US-A- 3 462 248

## Description

### Background of the Invention

### 1. Field of the Invention

This invention relates, in general, to a heat-resisting aluminum alloy which is high in mechanical strength not only at ordinary temperatures but also at high temperatures, and more particularly to the heat-resisting aluminum alloy suitable for the material of automotive engine component parts subjected to ordinary to high temperatures.

### 2. Description of the Prior Art

It is a recent tendency that improved fuel economy has been eagerly desired particularly in the field of automotive vehicles. As a measure for attaining the improved fuel economy, weight reduction of the automotive vehicles has been made by using light weight component parts made, for example, of aluminum alloy. Thus, aluminum alloy has been extensively used as the material of the automotive vehicle component parts, particularly of engine component parts.

However, it is difficult to employ usual aluminum alloy for the material of the engine component parts which are required to have a high mechanical strength throughout a wide temperature range from normal temperatures to about 250°C.

More specifically, so-called high strength aluminum alloy such as one whose designation number is 7075 has a good strength characteristics at normal temperatures but is sharply lowered in strength in a temperature range from normal temperatures to 200°C. In this regard, such high strength aluminum alloy is not suitable for the material of the component parts of automotive engines. The designation numbers of aluminium alloys mentioned hereinabove and hereinafter are adopted by the Aluminium Association in the United States of America.

Regarding so-called heat-resisting aluminium alloys such as one whose designation number is 2218, it is excellent in strength at high temperatures but is lower in strength at normal temperatures. As a result, such a heat-resisting aluminium alloy is also not suitable for the material of automotive engine component parts. Heat-resistant aluminium alloys comprising 2.2 to 6% manganese are disclosed in FR-A-1 370 542. These conventional heat-resistant aluminium alloys are based on the finding that aluminium-manganese alloys comprising 4% manganese up to 4% iron and up to 0.02% titanium can be processed by casting and have high mechanical strengths at temperatures of around 650°C. A typical alloy of this type having excellent mechanical properties at temperatures of higherthan 650°C consists of 3 to 9% manganese, 2.5 to 12% iron, 0.001 to 2.5% titanium, the balance being aluminium and impurities such as copper, zinc and magnesium.

It is the primary object of the present invention to provide an aluminium alloy which is excellent in mechanical strength (tensile strength, yield strength) both at ordinary temperatures and at high temperatures.

The above object is achieved by heat-resisting aluminium alloy consisting of more than 6 to 8% by weight manganese, from 0.5 to 2% by weight iron, from 0.03 to .05% by weight zirconium, from 2 to 5% by weight copper, the balance being aluminium and incidental impurities.

Preferred embodiments and further improvements of the invention are indicated in the sub-claims.

By virtue particularly of the lowered upper limit of content of manganese and iron and the increased content of copper, the aluminum alloy becomes high both in strength at ordinary and high temperatures and becomes suitable for the material of an article produced by using so-called atomization process in which molten metal of the parent metal is sprayed to obtain powder particles which will be finally compression-formed into a desired article.

In the inventive aluminium alloy, the upper limit of the added amount or content of manganese (Mn) and iron (Fe) is kept lower thereby to suppress crystallization of bulky phase and segregation of Mn compound, while increasing the added amount of content of copper (Cu) which is an additive element for improving mechanical strength throughout a wide temperature range from ordinary temperatures to about 250°C without affecting Mn compound. This make possible to obtain the heat-resisting aluminum which is high in mechanical strength both at ordinary temperatures and high temperatures without using quench solidification such as so-called splat cooling process which will complicate production processes thereafter.

The above-stated range of content of the components of the heat-resisting aluminum alloy of the present invention has been limited for the reasons discussed hereinafter.
Mn: more than 6 to 8% by weight (excluding a content of 6.0%).

Mn is an element effective for improving heat resistance and wear resistance of aluminium alloy. However, if the content of Mn is 6% or less, sufficient heat resistance cannot be obtained, while if it exceeds 8%, there occurs crystallization of the bulky phase and segregation of Mn compound at the cooling rate obtained by the atomization process. As a result, the content of Mn has been limited within the range from more than 6 to 8% by weight.
Fe: 0.5 to 2% by weight.

Fe is an element effective for improving high temperature stability of supersaturated solid solution (obtained by quenching) of AI-Mn alloy and fine Al-Mn intermetallic compound. However, if the content of Fe is less than 0.5%, such an effect cannot be obtained, while if it exceeds 2%, brittle phase of AI-Mn-Fe and Al-Fe is crystallized in the atomization process. As a result, the content of Fe has been limited within the range from 0.5 to 2% by weight.
Zr: 0.03 to 0.5% by weight.

Zr is an element effective for making fine crystal particles in addition for improving high temperature stability of supersaturated solid solution of Al-Mn alloy and fine Al-Mn intermetallic compound. However, the content of Zr is less than 0.03%, such an effect cannot be obtained, while if it exceeds 0.5%, there occurs enlargement of AI-Zr phase. As a result, the content of Zr has been limited within the range from 0.03 to 0.5% by weight.
Cu: 2 to 5% by weight.

Cu is an element which is effective for improving mechanical strength at ordinary temperatures and by which the heat-resisting aluminum alloy according to the present invention is most characterized. In other words, the present invention is intended to improve the mechanical strength in a wide temperature range from ordinary temperatures to 250°C without affecting Mn compound, by increasing the content of Cu in order to compensate a decrease of Mn, Fe content which decrease is made for the purpose of suppressing coarsening and segregation of Mn compound in powder form produced by the atomization process. It will be noted that if the content of Cu is less than 2%, the effect of strength improvement cannot be expected, while if it exceeds 5%, corrosion resistance of the aluminum alloy is degraded, accompanied by deteriorating the high temperature stability of the supersaturated solid solution of AI-Mn alloy and very fine Al-Mn intermetallic compound. As a result, the content of Cu has been limited within the range from 2 to 5% by weight.

Now, addition of silicon (Si) and magnesium (Mg) other than Cu is thinkable. However, if Si is added in a corresponding amount aiming the same degree strength improvement as in the case of Cu addition, Si is unavoidably contained in the form of a-AI(Fe,Mn)Si phase in Mn compound and therefore is less than Cu in strength improvement effect due to solid solution hardening and precipitation hardening.

Mg is an element which improves mechanical strength at ordinary temperatures by age hardening upon binding of Mg with Si. However, as stated above, Si tends to take the form a-AI(Fe, Mn)Si phase and therefore strength improvement due to the precipitation of M₉₂Si phase is degraded as compared with that due Cu addition.

In order to evaluate the heat-resisting aluminum alloy according to the present invention, Examples (Sample Nos. 1 to 5) of the present invention will be discussed hereinafter in comparison with Comparative Examples (Sample Nos. 6 to 12) which are out of the scope of the present invention. The chemical compositions of the Examples and Comparative Examples are shown in Table 1.

The aluminum alloys of Sample Nos fto 5 and of Sample Nos. 8 to 12 were prepared as follows: A binary alloy ingot containing A1 and an individual component other than Al, and an AI ingot were weighed and molten to be mixed with each other thereby to produce a parent metal having a chemical composition shown in table 1. Thereafter, the patent metal was molten in a melting furnace of an atomizing device, and the thus prepared molten metal was sprayed upon being superheated 150°C over the melting point of the parent metal, thereby obtaining atomized powder. The atomized powder having a particle size not larger than 120 mesh was used for preparing a specimen subjected to tests discussed below. Subsequently, the atomized powder was formed into a cylindrical shape under the compression of 3.5 KN/cm² to obtain a billet. The billet was then subjected to an extrusion process at a temperature lower than 400°C and at an extrusion ratio (the ratio between the cross-sectional areas of the billet and an extruded product) of 12:1. The extruded product was cut out into a predetermined shape to obtain the specimen for the tests.

The Sample Nos. 6 and 7 correspond to aluminum alloys whose designation numbers are 2218 and 7075, respectively. These were prepared as follows: The molten metal of the parent metal corresponding to each Sample No. was formed into an ingot for rolling which ingot thereafter underwent hot rolling. Subsequently, a product corresponding to Sample No. 6 was subjected to solid solution treatment at 510°C for 4 hours and to artificial aging treatment at 175°C for 4 hours, whereas a product corresponding to Sample No. 7 was subjected to solid solution treatment at 460°C for 4 hours and to artificial aging treatment at 120°C for 24 hours. Thereafter, each product were cut out into the predetermined shape to obtain each specimen for the tests.

Next, a tension test was conducted on each of the thus obtained specimens at an ordinary (or room) temperature and at 200°C, in which tension value measurement in test at 200°C was made after each specimen had been kept heated for 1 hour. The test result is shown in Table 2 in which Sample Nos. correspond to those in Table 1.

As shown in Table 2, all the Sample Nos. 1 to 5 aluminum alloys according to the present invention exhibit considerably higher tensile strengths at ordinary temperatures and at 200°C than the designation number 2218 heat-resisting aluminum alloy (Sample No. 6). Particularly, the strength at ordinary temperatures of the aluminum alloys according to the present invention can stand comparison with that of the designation number 7075 high strength aluminum alloy (Sample No. 7). Thus, it has been demonstrated that the aluminum alloy according to the present invention is excellent in strength at ordinary temperatures and at high temperatures.

The Sample Nos 8 and 9 aluminum alloys (Comparative Examples) whose Mn and Fe contents are less than those of the aluminum alloy of the present invention are slightly lower in strength at 200°C as compared with the aluminum alloy of the present invention. The Sample Nos. 10, 11 and 12 aluminum alloys (Comparative Examples) whose Mn and Fe contents are more than those of the aluminum alloy of the present invention are degraded in strength as compared with the aluminum alloy of the present invention because coarsening and segregation of Mn compound unavoidably occurs at the cooling rate obtained by the atomization process. Thus, the Sample Nos. 8 to 12 aluminum alloys have been confirmed to be inferior as compared with the aluminum alloy according to the present invention.

As will be appreciated from the above discussion, the aluminum alloy according to the present invention is a light alloy material which is excellent in mechanical strength both at ordinary temperatures and at high temperatures as compared with conventional aluminum alloys, so that it is widely applicable, for example, engine component parts which are required not only to be heat-resistant but also to be high in ordinary temperature strength, while achieving weight reduction of the component parts and an assembled product. Additionally, an article made of the aluminum alloy of the present invention can be produced with powder particles prepared by the atomization process, thus offering an advantage of omitting quench solidification such as troublesome splat cooling process.

## Claims

1. A heat-resisting aluminium alloy consisting of more than 6 to 8% by weight manganese, from 0.5 to 2% by weight iron, from 0.03 to 0.5% by weight zirconium, from 2 to 5% by weight copper, the balance being aluminium and incidental impurities.

2. Use of the aluminium alloy of claim 1 for the manufacture of a component part of an automotive engine.

3. A method for producing an article having improved strength at temperatures ranging from ordinary temperature to 250°C comprising preparing a parent metal having a composition as set forth in claim 1; melting said parent metal to obtain a melt of said parent metal; spraying said melt to obtain atomized powder particles; and forming said powder particles into a predetermined shape.

4. A method as claimed in claim 3, wherein the step of spraying is carried out in a condition where said molten is superheated 150°C over melting point of said parent metal.

5. A method as claimed in claim 4, further comprising the step of selecting powder particles having particle sizes smaller than 125pm (120 mesh) after step of spraying.

6. A method as claimed in claim 5, wherein the step of forming is carried out by compressing said powder particles under pressure of about 343N/mm² (3.5 tonf/cm²).

7. A method as claimed in claim 6, further comprising the step of extruding said formed powder particles into a predetermined shape after step of forming.

8. A method as claimed in claim 7, wherein the step of extruding is carried out at a temperature lower than 400°C.

## Patentansprüche

1. Wärmebeständige Aluminiumlegierung, bestehend aus mehr als 6 bis 8 Gew.-% Mangan, aus 0,5 bis 2 Gew.-% Eisen, aus 0,03 bis 0,5 Gew.% Zirconium, aus 2 bis 5 Gew.-% Kupfer, wobei der Rest Aluminium und zufällige Verunreinigungen sind.

2. Verwendung der Aluminiumlegierung nach Anspruch 1 zur Herstellung eines Komponententeils eines Kraftfahrzeugmotors.

3. Verfahren zur Herstellung eines Gegenstands mit verbesserter Festigkeit bei Temperaturen im Bereich von üblicher Temperature bis 250°C, bei dem ein Ausgangsmetall mit einer Zusammensetzung gemäß Anspruch 1 hergestellt wird, das Ausgangsmetall zur Herstellung einer Schmelze des. Ausgangsmetalls geschmolzen wird, die Schmelze zur Herstellung von Zerstäubten Pulverteilchen gesprüht wrid und die Pulverteilchen zu einer vorbestimmten Form geformt werden.

4. Verfahren nach Anspruch 3, worin die Sprühstufe in einem Zustand durchgeführt wird, wo die Schmelze 150°C über dem Schmelzpunkt des Ausgangsmetalls superwarmt wird.

5. Verfahren nach Anspruch 4, das weiterhin eine Stufe einschließt, bei der Pulverteilchen mit Teilchengrößen von weniger als weniger 125 um (120 mesh) nach der Sprühstufe ausgewählt werden.

6. Verfahren nach Anspruch 5, worin die Formungsstufe durchgeführt wird, indem die Pulverteilchen unter Druck von etwa 343 N/mm² (3,5 t/cm²) komprimiert werden.

7. Verfahren nach Anspruch 6, das weiterhin eine Stufe einschließt, bei der die gebildeten Pulverteilchen in eine vorbestimmte Form nach der Formungsstufe extrudiert werden.

8. Verfahren nach Anspruch 7, worin die Extrusionsstufe bei einer Temperatur von weniger als 400°C durchgeführt wird.

## Revendications

1. Alliage d'aluminium résistant aux températures élevées consistant en plus de 6 à 8% en poids de manganèse, de 0,5 à 2% en poids de fer, de 0,03 à 0,5% en poids zirconium, de 2 à 5% en poids de cuivre, le reste étant de l'aluminium et des impuretés accidentelles.

2. Utilisation de l'alliage d'aluminium de la revendication 1 pour la fabrication d'une pièce composante d'un moteur d'automobile.

3. Méthode de production d'un article ayant une meilleure résistance aux températures comprises entre la température ordinaire et 250°C consistant à préparer un métal parent ayant la composition indiquée à la revendication 1; à faire fondre ledit métal parent pour obtenir une fonte dudit métal parent; à pulvériser ladite fonte pour obtenir des particules pulvérulentes atomisées; et à donner auxdites particules pulvérulentes une forme prédéterminée.

4. Méthode selon la revendication 3, où l'étape de pulvériser est efectuée dans une condition où ledit produit fondu est surchauffé à 150°C par rapport au point de fusion dudit métal parent.

5. Méthode selon la revendication 4, comprenant de plus l'étape de choisir des particules pulvérulentes ayant des granulométries plus petites que 125 pm (maille 120) après l'étape de pulvérisation.

6. Méthode de la revendication 5, où l'étape de mise en forme est effectuée en comprimant lesdites particules pulvérulentes sous une pression d'environ 343 N/mm² (3,5 tonnes force/cm²).

7. Méthode selon la revendication 6, comprenant de plus l'étape d'extruder lesdites particules pulvérulentes formées à une forme prédéterminée après l'étape de mise en forme.

8. Méthode selon la revendication 7, où l'étape d'extruder est effectuée à une température inférieure à 400°C.
